



US011801702B2

(12) **United States Patent**  
**Boxhammer**

(10) **Patent No.:** **US 11,801,702 B2**  
(45) **Date of Patent:** **Oct. 31, 2023**

(54) **COATING COMPOSITION, HEAT-SENSITIVE RECORDING LAYER, HEAT-SENSITIVE RECORDING MATERIAL, AND CORRESPONDING USES AND METHODS**

(71) Applicant: **Mitsubishi HiTec Paper Europe GmbH**, Bielefeld (DE)

(72) Inventor: **Claas Boxhammer**, Herford (DE)

(73) Assignee: **MITSUBISHI HITEC PAPER EUROPE GMBH**, Bielefeld (DE)

(\*) Notice: Subject to any disclaimer, the term of this patent is extended or adjusted under 35 U.S.C. 154(b) by 526 days.

(21) Appl. No.: **16/966,148**

(22) PCT Filed: **Jan. 31, 2019**

(86) PCT No.: **PCT/EP2019/052347**

§ 371 (c)(1),  
(2) Date: **Jul. 30, 2020**

(87) PCT Pub. No.: **WO2019/149805**

PCT Pub. Date: **Aug. 8, 2019**

(65) **Prior Publication Data**

US 2021/0031551 A1 Feb. 4, 2021

(30) **Foreign Application Priority Data**

Jan. 31, 2018 (DE) ..... 10 2018 102 177.1

(51) **Int. Cl.**

**B41M 5/333** (2006.01)  
**B41M 5/337** (2006.01)  
**B41M 5/327** (2006.01)

(52) **U.S. Cl.**

CPC ..... **B41M 5/3333** (2013.01); **B41M 5/3275** (2013.01); **B41M 5/3375** (2013.01); **B41M 2205/04** (2013.01); **B41M 2205/38** (2013.01)

(58) **Field of Classification Search**  
CPC .. B41M 5/323; B41M 5/3275; B41M 5/3333;  
B41M 5/3375; B41M 2205/04; B41M  
2205/38

See application file for complete search history.

(56) **References Cited**

U.S. PATENT DOCUMENTS

10,160,245 B2 \* 12/2018 Horn ..... B41M 5/3333

FOREIGN PATENT DOCUMENTS

DE 3544758 7/1986  
DE 3636222 4/1987

(Continued)

OTHER PUBLICATIONS

Office Action of the corresponding German Patent Application No. 10 2018 102 177.1.

(Continued)

*Primary Examiner* — Gerard Higgins

(74) *Attorney, Agent, or Firm* — Cozen O'Connor

(57) **ABSTRACT**

A coating composition for producing a heat-sensitive recording material and to a corresponding heat-sensitive recording layer. The coating composition includes one or more color developers, one or more dye precursors, one or more specific fatty acid amides, and one or more (additional) specific sensitizers. A heat-sensitive recording material including a carrier substrate and a heat-sensitive recording layer, to the use of specific fatty acid amides in order to increase the grease resistance of a heat-sensitive recording material or a heat-sensitive recording layer, and to a method for producing a heat-sensitive recording material or a heat-sensitive recording layer.

**16 Claims, 4 Drawing Sheets**



(56)

**References Cited**

FOREIGN PATENT DOCUMENTS

|    |                    |               |
|----|--------------------|---------------|
| DE | 10241903           | 3/2004        |
| DE | 102004004204       | 8/2005        |
| DE | 102008007596       | 8/2009        |
| DE | 102014107567       | 11/2015       |
| DE | 102015104306       | 9/2016        |
| DE | 112015000518       | 10/2016       |
| EP | 2923851            | 9/2015        |
| EP | 3000608            | 3/2016        |
| JP | 2005288743         | 10/2005       |
| JP | 2012-504442        | 11/2012       |
| WO | WO 9843824         | 10/1998       |
| WO | WO-2015181291 A1 * | 12/2015 ..... |
| WO | WO 2018065328      | 4/2018        |

OTHER PUBLICATIONS

DIN 53107 "Testing of Paper and Board—Determination of The Smoothness By The Bekk Method", May 2016.

DIN EN ISO 787-5 "General Methods of Test For Pigments and Extenders—Part 5: Determination of Oil Absorption Value", Oct. 1995.

\* cited by examiner



Fig. 1

Fig. 2







Fig. 4

## 1

**COATING COMPOSITION, HEAT-SENSITIVE RECORDING LAYER, HEAT-SENSITIVE RECORDING MATERIAL, AND CORRESPONDING USES AND METHODS**

**CROSS REFERENCE TO RELATED APPLICATIONS**

This is a U.S. national stage of Application No. PCT/EP2019/052347 filed Jan. 31, 2019. Priority is claimed on German Application No. DE 10 2018 102 177.1 filed Jan. 31, 2018 the content of which is incorporated herein by reference.

**BACKGROUND OF THE INVENTION**

**1. Field of the Invention**

The present invention relates to a coating composition for producing a heat-sensitive recording material and also to a corresponding heat-sensitive recording layer. The coating composition comprises one or plural color developers, one or plural dye precursors, one or plural specific fatty acid amides, and one or plural (further) specific sensitizers. The present invention further relates to a heat-sensitive recording material comprising a carrier substrate and a heat-sensitive recording layer of the invention. The present invention relates, moreover, to the use of specific fatty acid amides for increasing the grease resistance of a heat-sensitive recording material or a heat-sensitive recording layer. The present invention also relates to a method for producing a heat-sensitive recording material of the invention or a heat-sensitive recording layer.

**2. Description of Related Art**

Heat-sensitive recording materials (e.g., for direct thermal printing applications) which have a heat-sensitive, color-forming recording layer applied on a carrier substrate have been known for many years and are enjoying high popularity. One of the reasons for this popularity is that the use of said materials is associated with the advantage that the color-forming components are contained in the recording material itself and it is therefore possible to use printers free from toner cartridges and ink cartridges. There is therefore no need to purchase and/or fill cartridges of ink or of toner. Accordingly, this innovative technology has become established largely across the board particularly in public transport and in retail.

In a coating composition for producing a heat-sensitive recording material, and in heat-sensitive recording layers of customary recording materials, there is a dye precursor and there is a color developer. On imagewise heating of the heat-sensitive recording layer by a suitable imaging tool, as for example a thermal head or thermal rod, a laser beam, or the like, to a suitable temperature, the coating melts, softens, or sublimes, with the dye precursor and the color developer contacting one another, reacting with one another, and, as a consequence of this chemical reaction, almost immediately forming an image with high color density on the recording material. Preference has been given in recent times, and is also given in the context of the present invention, to the use of nonphenolic color developers.

A heat-sensitive recording material is generally produced by using a coating machine to apply a coating composition for generating a heat-sensitive recording layer to a suitable carrier substrate, i.e., a suitable paper web, a polymeric film,

## 2

or a corresponding material, then drying the coating composition to give the heat-sensitive recording layer, and optionally smoothing this layer by a calendar. In addition to the heat-sensitive recording layer, preliminary coatings, intermediate coatings and/or finishing coatings may be applied either to one side or to both sides of the recording material. This is also true of a heat-sensitive recording material of the invention.

A coating composition for producing a heat-sensitive recording layer or a heat-sensitive recording material is frequently produced (and is also produced in the context of the present invention) by grinding and dispersing, separately, at least one dye precursor, at least one color developer, and at least one sensitizer to a suitable particle size by bead mills or ball mills, in water or a suitable solvent. The fine dispersions produced accordingly are mixed in the desired ratio with the binders, pigments, lubricant, and release agents, and also with the other customary auxiliaries, which are used together with these fine dispersions as the coating composition for the heat-sensitive recording layer.

DE 10 2014 107 567 B3, according to its independent claim 1, concerns a heat-sensitive recording material comprising a carrier substrate and also a heat-sensitive, color-forming layer comprising at least one color former (i.e., dye precursor), at least one phenol-free color developer, and at least one sensitizer. Paragraph [0014] discloses N-[2-(3-phenylureido)phenyl]benzenesulfonamide (NKK) as color developer. Paragraph [0024] discloses a list of sensitizers which includes—alongside a multiplicity of other compounds—stearamide, 1,2-diphenoxylethane, and 1,2-di(3-methylphenoxy)ethane.

DE 10 2004 004 204 A1, according to its independent claim 1, concerns a heat-sensitive recording material, having a substrate and a heat-sensitive recording layer which comprises a sensitizer, pigment, binder, at least one color former (i.e., dye precursor) and also a phenolic color developer and at least one further organic color developer, the phenolic color developer being selected from the group of the bis(hydroxyphenyl) compounds, and at least one of the further color developers being a urea-urethane compound.

DE 35 44 758 C2, according to its independent claim 1, concerns a paper coating slip which comprises a polyvinyl alcohol resin which contains acetoacetyl groups.

DE 36 36 222 A1, according to its independent claim 1, concerns a heat-sensitive paper set which is able to develop a black image having excellent oil resistance and light stability.

WO 98/43824 A1, according to its independent claim 1, concerns a heat-sensitive recorded sheet having a substrate, a heat-sensitive recording layer comprising color formers (i.e., dye precursors) and color acceptors, and a pigment-containing protective layer which is formed on the recording layer and which comprises a mixture of water-soluble binder and water-insoluble binder.

DE 10 2008 007 596 A1, according to its independent claim 1, relates to a method for producing a recording material, comprising the step of applying a coating which comprises constituents protecting a coating applied in a preceding step from disadvantageous alteration, and comprises a self-crosslinking polyvinyl alcohol in combination with a polyurethane resin.

DE 102 41 903 A1, according to its independent claim 1, concerns a method for producing a layered, heat-sensitive recording material in web form, the recording material comprising at least one substrate, a heat-sensitive recording

layer comprising color formers (i.e., dye precursors) and color acceptors, and a protective layer formed on the recording layer.

DE 11 2015 000 518 T5 (Mitsubishi Paper Mills Limited), according to its independent claim 1, concerns a thermal recording material having a heat-sensitive recording layer on a paper carrier, said layer comprising a colorless or slightly colored color origin substance and a developer which reacts with the color origin substance on heating and converts the color origin substance into its color form; the paper carrier comprises a mass fraction of 0.25 to 1.0% of a neutral rosin size, based on the cellulose solids content, in combination with calcium carbonate and aluminum sulfate; and the developer has a phenylureido group in its molecule. The developer in certain embodiments is N-[2-(3-phenylureido)phenyl]benzenesulfonamide. A variety of compounds are listed as suitable sensitizers; alongside a multiplicity of other compounds, the list also embraces monostearamide 1,2-diphenoxymethane, and 1,2-bis(3-methylphenoxy)ethane.

JP 2012-504442 (Hatsume Suishin Kyokai Kokai Giho; published Nov. 22, 2012) discloses a RECORDING MATERIAL PRODUCED USING NON PHENOL COMPOUND (English translation of the title as per translation from the German Opposition procedure relating to the patent DE 10 2014 107 567 B3).

EP 3 000 608 A1, according to its independent claim 1, concerns a heat-sensitive recording material comprising a heat-sensitive recording layer on a carrier, the heat-sensitive recording layer comprising at least one leuco dye and as developer a sulfonamide compound. According to alternative (b) of claim 1, the heat-sensitive recording layer may further comprise a saturated fatty acid amide. According to claim 5, the heat-sensitive recording material may additionally comprise a sensitizer.

DE 10 2015 104 306 A1, according to its independent claim 1, concerns a heat-sensitive recording material comprising a carrier substrate and also a heat-sensitive, color-forming layer comprising at least one color former and at least one phenol-free color developer.

## SUMMARY OF THE INVENTION

With the aim of improving heat-sensitive recording materials, especially in the context of their use as tickets or lottery slips, with regard to their resistance to environmental effects such as heat, moisture, and chemicals, there is an ongoing interest in continual onward development of the underlying chemistry and the production technology for generating such recording materials and the coating compositions and recording layers on which these materials are based.

Increasingly in the recent past there have arisen concerns regarding the environmental compatibility particularly of certain (bis)phenolic color developers. Recently then, among the color developers, for example, the well-known components that have been subjects of exceptionally good scientific study, and are known in the form of

bisphenol A, namely 2,2-bis(4-hydroxyphenyl)propane, and

bisphenol S, namely 4,4-dihydroxydiphenyl sulfone,

having increasingly become a focus of public criticism and for that reason have been replaced, for example, completely or partly by NKK, namely N-[2-(3-phenylureido)phenyl]benzenesulfonamide, of the formula



The present invention relates to such a coating composition for producing a heat-sensitive recording material and also to a heat-sensitive recording layer, each comprising NKK as color developer.

In particular there is an ongoing command for further heat-sensitive recording materials for a wide variety of different uses; in view of the high sales volumes of these materials in a keenly fraught market, these materials must be producible at low cost and must therefore possess a simple construction. One particular challenge here is that in the course of their typical uses as gaming tickets, entry tickets, travel tickets, pay parking tickets, and so on, heat-sensitive recording materials are exposed to a multiplicity of different ambient influences, such as moisture, heat, or chemicals.

For instance, during their normal use, heat-sensitive recording materials may come into contact with a multiplicity of different substances that can affect the durability of the thermal printout. These substances, besides water and organic solvents, also include fats and oils that are present, for example, in hand care products and which may become transferred to the heat-sensitive recording material on touching said material. There is therefore also a need for grease resistance on the part of the recording material, so that the recorded image is not destroyed on contact with oily or greasy substances, such as with fatty constituents in haircare products or hand creams, or from skin deposits.

As well as durability to chemicals that may come into contact with the heat-sensitive recording materials, said materials must also be very durable toward thermal influences. On the one hand, the heat-sensitive recording material should be able to be printed easily without excessive energy, so that little energy is consumed in mobile applications, for example. On the other hand, the printed image is to last after printing, and the action of heat should cause neither the printed image to fade nor the unprinted background to discolor, resulting in the print ceasing to be legible. Paid parking tickets which, once printed, are displayed behind the windshield and thereby become exposed in the summer to high temperatures and direct sunlight, are an example of where thermal durability is very much relevant.

Similarly with tickets such as concert tickets or flight tickets, which are frequently produced a long time in advance, or with purchase receipts, which are needed as proof of purchase over a long guarantee period, the long-term durability of the heat-sensitive recording material is very important.

Particularly in view of the potential toxicity of (bis)phenolic chemicals, the development of new, heat-sensitive recording materials ought additionally to minimize or negate entirely the use of (bis)phenolic color developers and to instead give preference to the use of (bis)phenol-free color developers, such as NKK, for instance.

In-house studies have shown that the use of NKK as a color developer within coating compositions and heat-sensitive recording layers of heat-sensitive recording materials, in comparison with conventional, (bis)phenol-containing

color developers, has the disadvantageous result of a reduction in the grease resistance of the resulting heat-sensitive recording material. According to the in-house studies, the use of NKK resulted in greatly accelerated retrograde development of color after the direct contact of the heat-sensitive recording material (in a thermal paper) with fats and oils, thereby severely restricting the applications of NKK-containing, heat-sensitive recording materials without a topcoat and so being at the expense of a simple construction of such recording materials.

A primary object of one aspect of the present invention was to specify a coating composition comprising N-[2-(3-phenylureido)phenyl]benzenesulfonamide (NKK) of the formula



as color developer for producing a heat-sensitive recording material, and also a corresponding heat-sensitive recording layer, which is distinguished by only slow retrograde development of color after direct contact of fats and oils with the recording material provided with a recorded image (i.e., printed). A further object was to specify a corresponding heat-sensitive recording material and also methods for producing said material.

The heat-sensitive recording material to be specified ought also to possess high thermal response sensitivity, high background whiteness and high image density, and an improved durability of the recording generated thereon by means of heat exposure with respect to humidity or heat; this applies corresponding to the coating composition that is to be specified and to the recording layer that is to be specified. The heat-sensitive recording materials ought preferably to exhibit long-term aging even at high temperatures (40 to 60° C.) and possibly high atmospheric humidity.

Further objects are apparent from the description below and from the claims.

The subject matter of the invention is defined in the appended claims and in the description hereinafter.

According to a first aspect of the invention, a coating composition for producing a heat-sensitive recording material, and, respectively, by a heat-sensitive recording layer, comprises

one or plural color developers, said one or at least one of the plural color developers being a compound of the formula (I)



one or plural dye precursors,

one or plural fatty acid amides each having a number of carbon atoms in the range from 16 to 24, as sensitizer, one or more compounds selected from the group consisting of 1,2-diphenoxymethane (DPE) and ethylene glycol m-tolyl ether (EGTE),

5 the ratio of the total mass of fatty acid amides having a number of carbon atoms in the range from 16 to 24 to the total mass of compounds selected from the group consisting of 1,2-diphenoxymethane and ethylene glycol m-tolyl ether in 10 the coating composition or the heat-sensitive recording layer being in the range from 4:1 to 1.2:1.

The compound of the formula (I) is, as already indicated earlier on above, NKK, i.e., N-[2-(3-phenylureido)phenyl]benzenesulfonamide.

15 One aspect of the invention also relates to a corresponding heat-sensitive recording material comprising a carrier substrate and

20 a heat-sensitive recording layer of the invention (as defined above and below, and in the claims).

One aspect of the invention uses a fatty acid amide having a number of carbon atoms in the range from 16 to 24 or of a mixture of plural fatty acid amides each having a number of carbon atoms in the range of 16 to 24, preferably through 25 the use of octadecanamide and/or N-(hydroxymethyl)octadecanamide, for increasing the grease resistance of a heat-sensitive recording material or a heat-sensitive recording layer, comprising

one or plural color developers, said one or at least one of the plural color developers being a compound of the formula (I)



one or plural dye precursors, and

as sensitizer, one or more compounds selected from the group consisting of 1,2-diphenoxymethane (DPE) and ethylene glycol m-tolyl ether (EGTE),

35 the ratio of the total mass of fatty acid amides having a number of carbon atoms in the range from 16 to 24 to the total mass of compounds selected from the group consisting of 1,2-diphenoxymethane and ethylene glycol m-tolyl ether in the heat-sensitive recording material or the heat-sensitive recording layer being in the range from 4:1 to 1.2:1.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 963

having the following steps:  
providing or producing

a carrier substrate with interlayer disposed thereon  
and also

a coating composition of the invention (as defined above and below, and in the claims),  
applying the coating composition to the interlayer,  
drying the applied coating composition, to give a heat-sensitive recording layer which is present together with the carrier substrate and the interlayer in the heat-sensitive recording material.

The compound having the formula (I) is already known and is disclosed for example in EP 2 923 851 A1 or the aforementioned DE 10 2014 107 567 B3. It corresponds to the compound already identified in the text above as NKK.

One aspect of the invention is based on the surprising experimental finding that a coating composition for producing a heat-sensitive recording material, or a corresponding heat-sensitive recording layer, which as color developer comprises a compound of formula (I)



(that is NKK, i.e., N-[2-(3-phenylureido)phenyl]-benzenesulfonamide)

and further comprises one or plural dye precursors, possesses a particularly and unexpectedly high grease resistance if the coating composition or the heat-sensitive recording layer comprise at the same time

one or more fatty acid amides each having a number of carbon atoms in the range from 16 to 24

and

as sensitizer, one or more compounds selected from the group consisting of 1,2-diphenoxymethane (DPE) and ethylene glycol m-tolyl ether (EGTE),

and preferably

the ratio of the total mass of fatty acid amides having a number of carbon atoms in the range from 16 to 24 to the total mass of compounds selected from the group consisting of 1,2-diphenoxymethane and ethylene glycol m-tolyl ether in the coating composition or the heat-sensitive recording layer is in the range from 4:1 to 1.2:1.

The increased grease resistance here can presumably be attributed to a synergistic effect between fatty acid amide and the sensitizer used. At least, in experimental studies in house, it has emerged that in coating compositions of the invention comprising either octadecanamide (stearamide) or N-(hydroxymethyl)octadecanamide and also, as sensitizer, either 1,2-diphenoxymethane (DPE) or ethylene glycol m-tolyl ether (EGTE), the total mass of octadecanamide or N-(hydroxymethyl)octadecanamide and DPE or EGTE being kept constant in each case but the mass ratio varied, the grease resistance ascertained experimentally in each case was not merely attributable additively to the performance of the individual octadecanamide or N-(hydroxymethyl)octadecanamide and DPE or EGTE constituents. Surprisingly, instead, it emerged that the grease resistance in the mixtures was superadditive. In-house studies on the grease resistance

were carried out according to a test method which is specified below under the heading "Determining the resistance of heat-sensitive recording materials to lanolin".

Commercially available lanolin (as used in the in-house studies on grease resistance) constitutes a mixture which is obtained by melting together 65 mass fractions of woolwax, 20 mass fractions of water, and 15 mass fractions of low-viscosity paraffin. Woolwax (wool grease, *adeps lanae*, INCI designation: lanolin, E 913) is the secretion of the sebaceous glands of the sheep. It is got by extraction of ovine fleeces with isopropanol. The name lanolin derives from the Latin *lana* for wool and *oleum* for oil.

In the present text—as in a great many documents from the prior art—a series of designations, synonymous with one another and identical in content, are used for substances that are the same in each case. Set out below for a series of a total of six substances or substance classes are those synonymous designations which are used in the context of the present text and in documents from the prior art.

1. The compound of the formula (I)



is identified in the present text as NKK or as N-[2-(3-phenylureido)phenyl]benzenesulfonamide; the same compound is identified in DE 10 2014 107 567 B3 likewise as N-[2-(3-phenylureido)phenyl]benzenesulfonamide, and as phenylureidophenylbenzenesulfonamide. In the as yet unpublished application PCT/EP2017/074875, the designations N-[2-(phenylcarbamoyl)amino]phenyl]benzenesulfonamide and N-[2-(3-phenylureido)phenyl]-benzenesulfonamide are used for the same substance. Compounds with the CAS number 215917-77-4 and the EC No. 806-543-7 are also identified as NKK.

2. Ethylene glycol m-tolyl ether is also identified as EGTE in the present text; the same compound is identified in DE 10 2014 107 567 B3 as 1,2-di(3-methylphenoxy)ethane. The application PCT/EP2017/074875 for this same substance uses the designations 1,2-di(m-methylphenoxy)ethane and 1,2-bis(3-methylphenoxy)ethane. The compound with the CAS number 54914-85-1 is also identified as ethylene glycol m-tolyl ether.

3. Octadecanamide is identified in DE 10 2014 107 567 B3 as stearamide or as stearic acid amide. The application PCT/EP2017/074875 likewise uses the designation stearamide for the same substance. The compound with the CAS number 124-26-5 is also identified as octadecanamide.

4. Benzyl 2-naphthyl ether is also identified in the present text as benzyl naphthyl ether; the same compound is identified in DE 10 2014 107 567 B3 as 2-benzylxynaphthalene. The compound with the CAS number 613-62-7 is also identified as benzyl 2-naphthyl ether.

5. The substance class of the dye precursors is referred to in DE 10 2014 107 567 B3 as color formers. The application PCT/EP2017/074875 uses the designation dye precursors and also the designation color formers for the same substance class.

6. The substance class of the sensitizers is referred to in DE 10 2014 107 567 B3 as sensitizing agents.

In the aforementioned document DE 10 2014 107 567 B3 there are no indications that the fatty acid amide employed therein, stearamide (octadecanamide), might interact synergistically with one or more of the further sensitizing agents (sensitizers) specified in said document. In light of this fact, the technical effects achievable with the present invention and the findings on which the invention is based are particularly surprising.

A coating composition of the invention or a heat-sensitive recording layer of one aspect of the invention (as defined above and in the claims) preferably comprises one or more constituents from the group consisting of

further sensitizers,  
pigments,  
dispersants,  
antioxidants,  
release agents,  
defoamers,  
light stabilizers,  
and  
brighteners.

A coating composition of one aspect of the invention or heat-sensitive recording layer of one aspect of the invention comprises in every case a sensitizer, namely in accordance with one aspect of the invention at least one or plural compounds from the group comprising 1,2-diphenoxymethane (DPE) and ethylene glycol m-tolyl ether (EGTE). The one or plural fatty acid amides present in accordance with one aspect of the invention and each having a number of carbon atoms in the range from 16 to 24 are likewise understood by many experts to be sensitizers. In addition, however, there are preferably one or plural further sensitizers present.

A sensitizer in a heat-sensitive recording layer is first melted during the supply of heat during the printing operation, and the melted sensitizer dissolves the color formers and color developers present alongside one another and/or lowers the melting temperature of the color formers and color developers, to bring about a color development reaction. The sensitizer itself does not take part in the color development reaction.

A "further sensitizer" comprehends substances which (likewise) serve for adjusting the melting temperature (color development temperature) of the heat-sensitive recording layer and with which it is possible preferably to set a melting temperature of <100° C., preferably in the range from around 70 to 80° C., without the sensitizers themselves participating in the color development reaction.

Employed preferably as further sensitizers are, for example, fatty acid salts, fatty acid esters, and fatty acid amides (e.g., zinc stearate, palmitamide, oleamide, lauramide, ethylene- and methylenebisstearamide, methylolstearamide), naphthalene derivatives, biphenyl derivatives, and phthalates and terephthalates.

Particularly preferred is a coating composition of one aspect of the invention or a heat-sensitive recording layer of one aspect of the invention, wherein the further sensitizer is selected from the group consisting of 2-(2H-benzotriazol-2-yl)-p-cresol, 2,2'-bis(4-methoxyphenoxy)diethyl ether, 4,4'-diallyloxydiphenyl sulfone, 4-acetylacetophenone, 4-benzylbiphenyl, acetoacetanilide, benzyl 2-naphthyl ether, benzyl naphthyl ether, benzyl 4-(benzyloxy)benzoate, benzyl paraben, bis(4-chlorobenzyl) oxalate ester, bis(4-methoxyphenyl) ether, dibenzyl oxalate, dibenzyl terephthalate, dimethyl terephthalate, dimethyl sulfone, diphenyl

adipate, diphenyl sulfone, ethylenebisstearamide, fatty acid anilides, m-terphenyl, N-methylolstearamide, N-stearylurea, N-stearylstearamide, p-benzylbiphenyl, phenyl benzene-sulfonate ester, salicylanilide, and  $\alpha,\alpha'$ -diphenoxylxylene, particular preference being given to benzyl naphthyl ether and diphenyl sulfone.

Likewise preferred as further sensitizers for use in a coating composition of one aspect of the invention or in a heat-sensitive recording layer of one aspect of the invention 10 are the sensitizers disclosed in paragraphs [0059] to [0061] of EP 2 923 851 A1. Particularly preferred is the use of one or plural further sensitizers, wherein the respective sensitizer has a melting point in the range from 60° C. to 140° C., preferably a melting point in the range from 60° C. to 100° 15 C.

As well as sensitizers, a coating composition of one aspect of the invention or a heat-sensitive recording layer of one aspect of the invention preferably also comprises one or more constituents from the group consisting of pigments, 20 dispersants, antioxidants, release agents, defoamers, light stabilizers, and brighteners. Each of these components is used preferably in an amount with a mass fraction of 0.01 to 15%, more particularly—except for defoamer—0.1 to 15%, preferably 1 to 10%, based on the total solids fraction of the 25 coating composition of the invention or of the heat-sensitive recording layer. When defoamer is used in a coating composition of one aspect of the invention or a heat-sensitive recording layer of the invention, the defoamer is present preferably in amounts with a mass fraction of 0.03 to 0.05%, 30 based on the total solids fraction of the coating composition of the invention or of the heat-sensitive recording layer of one aspect of the invention.

A heat-sensitive recording layer of one aspect of the invention can of course be shielded by the disposition of a 35 concealing protective layer in such a way as to afford protection against external influences. The disposition of such a protective layer, however, is generally unnecessary in the context of one aspect of the present invention and hence also not preferred. Because of the selection and combination 40 of fatty acid amides each having a number of carbon atoms in the range from 16 to 24 with a sensitizer from the group consisting of DPE and EGTE, indeed, the coating composition of one aspect of the invention and the heat-sensitive recording layer of one aspect of the invention are already 45 equipped in such a way as to afford a thermal printout on a heat-sensitive recording layer of one aspect of the invention, which, indeed, may in particular be a constituent of a heat-sensitive recording material of the invention, with outstanding resistance to substances selected from the group 50 consisting of water, alcohols, fats, oils, and mixtures thereof, and particularly with resistance to fats and oils, even without a protective layer.

A coating composition of one aspect of the invention or a 55 heat-sensitive recording layer of the invention comprises a compound of the formula (I) (that is, NKK). A compound of the formula (I) is already known and is described for example in EP 2 923 851 A1. It has emerged, however, that the compound of the formula (I) may be present in two different crystalline forms. The two crystalline forms have 60 different physical properties, which may have effects on the properties of the coating composition of one aspect of the invention, of the heat-sensitive recording layer of one aspect of the invention, and of the heat-sensitive recording material of one aspect of the invention.

65 A first crystalline form of the compounds with the formula (I) has a melting point of around 158° C., whereas a second crystalline form of the compounds with the formula (I) has

a melting point of 175° C. In connection with heat-sensitive recording materials, the only description in the literature to date has been of the compound with the formula (I) which is the crystalline form having a melting point of around 158° C. (cf., for example, EP 2 923 851 A1 paragraph [0084]). Neither the preparation nor the use of the crystalline form of the compounds with the formula (I) having a melting point of around 175° C., as used in accordance with one aspect of the invention, have been described in the literature published to date; cf., however, the application PCT/EP2017/074875. It must therefore be assumed that in accordance with the published prior art, the crystalline form of the compound with the formula (I) having a melting point of around 158° C. has always been used, even if the melting point is not explicitly mentioned in the corresponding document. The crystalline form of the compound of the formula (I) having a melting point of 175° C., as used in accordance with the invention, has recently become available commercially as well.

Preferred in accordance with one aspect of the invention, therefore, are a coating composition of the invention, a heat-sensitive recording layer of the invention, and a heat-sensitive recording material of the invention, wherein the crystalline form of the compound of the formula (I) exhibits a (preferably endothermic) transition at a temperature between 170° C. and 178° C., preferably between 173° C. and 177° C., more preferably between 174° C. and 176° C., determined by means of differential scanning calorimetry (DSC) at a heating rate of 10 K/min.

Both crystalline forms of the compounds having the formula (I) may likewise be distinguished from one another in the IR absorption spectrum. Particularly characteristic in the case of the crystalline form of the compounds having the formula (I), used in accordance with the invention, is an absorption band in the IR spectrum at  $3401\pm20\text{ cm}^{-1}$ . In the case of the crystalline form of the compounds having the formula (I) that has a melting point of around 158° C., this band is absent, there being instead a band at each of  $3322$  and  $3229\text{ cm}^{-1}$ .

Preferred in accordance with one aspect of the invention is a heat-sensitive recording material, wherein the crystalline form of the compound of the formula (I) in the IR spectrum has absorption bands at  $689\pm10\text{ cm}^{-1}$ ,  $731\pm10\text{ cm}^{-1}$ ,  $1653\pm10\text{ cm}^{-1}$ ,  $3364\pm20\text{ cm}^{-1}$ , and  $3401\pm20\text{ cm}^{-1}$ .

Preferred in accordance with one aspect of the invention are a coating composition of the invention, a heat-sensitive recording layer of the invention, and, respectively, a heat-sensitive recording material of the invention, wherein the IR absorption spectrum of the crystalline form of the compound of the formula (I) coincides substantially with the IR absorption spectrum depicted in FIG. 1a), 2a) and/or 3a).

The two crystalline forms of the compounds having the formula (I) may likewise be distinguished from one another in the X-ray powder diffractogram. Preferred in accordance with one aspect of the invention are a coating composition of the invention, a heat-sensitive recording layer of the invention, and a heat-sensitive recording material of the invention, wherein the crystalline form of the compound of the formula (I) has an X-ray powder diffractogram having diffraction reflections at  $\vartheta/20$  values of  $10.00\pm0.20$ ,  $11.00\pm0.20$ ,  $12.40\pm0.20$ ,  $13.80\pm0.20$ , and  $15.00\pm0.20$ .

Preferred in accordance with one aspect of the invention are a coating composition of the invention, a heat-sensitive recording layer of the invention, and a heat-sensitive recording material of the invention, wherein the crystalline form of the compound of the formula (I) has an X-ray powder

diffractogram which substantially coincides with the X-ray powder diffractogram depicted in FIG. 4b).

In-house studies worked predominantly with a crystalline form of the compound of the formula (I) that in the IR spectrum has an absorption band at  $3401\pm20\text{ cm}^{-1}$  and/or has a melting point of 175° C. and/or has a transition at a temperature between 170° C. and 178° C., determined by differential scanning calorimetry (DSC) at a heating rate of 10 K/min, and/or in the X-ray powder diffractogram has diffraction reflections at  $\vartheta/20$  values of at least  $10.00\pm0.20$ ,  $11.00\pm0.20$ ,  $12.40\pm0.20$ ,  $13.80\pm0.20$ , and  $15.00\pm0.20$ . The use of such a compound of the formula (I) is somewhat preferred for all aspects of the present invention. A coating composition of one aspect of the invention and also a heat-sensitive recording layer of the invention preferably comprise pigments. The pigments may be organic pigments, inorganic pigments, or a mixture of organic pigments and inorganic pigments.

A coating composition of one aspect of the invention or a heat-sensitive recording layer of the invention (as defined above, preferably as identified above as being preferred) is preferred, wherein said one or one of the plural fatty acid amides having a number of carbon atoms in the range from 16 to 24 is octadecanamide (stearamide; stearic acid amide). Octadecanamide is chemically compatible with the compound of the formula (I) (NKK) and with sensitizers from the group consisting of 1,2-diphenoxylethane (DPE) and ethylene glycol m-tolyl ether (EGTE). As the pure substance, octadecanamide possesses a melting point of 109° C. and it is therefore an outstanding sensitizer (cf. the corresponding use according to DE 10 2014 107 567 B3); it does not itself participate in the color development reaction. The capacity of octadecanamide (and other fatty acid amides having a number of carbon atoms in the range from 16 to 24) for synergistic interactions with DPE and/or EGTE was hitherto unknown from the prior art. Likewise preferred is the use of N-(hydroxymethyl)octadecanamide as fatty acid amide.

Preference is given to a coating composition of one aspect of the invention and to a heat-sensitive recording layer of one aspect of the invention, wherein octadecanamide or N-(hydroxymethyl)octadecanamide is used in combination with DPE and/or EGTE in such a way that the color reaction can take place at an exposure temperature (color development temperature) of as low as 100° C. Because octadecanamide possesses a melting point of 109° C. or N-(hydroxymethyl)octadecanamide possesses a melting point of >107° C. but EGTE possesses a melting point in the range from 96 to 100° C. and diphenoxylethane a melting point in the range from 94 to 96° C., the actual sensitizing performance in recording layers or coating compositions of the invention formulated in this way is primarily attributable to the presence of DPE or EGTE. The primary function of the octadecanamide in such a formulation, therefore, is of achieving and/or ensuring the desired grease resistance through synergistic interaction with DPE and/or EGTE. The desired grease resistance is achieved and/or ensured analogously, in a further configuration according to the invention, through synergistic interaction of N-(hydroxymethyl)octadecanamide with DPE and/or EGTE.

In a preferred coating composition of one aspect of the invention or heat-sensitive recording layer of one aspect of the invention, the ratio of the mass of the compound of the formula (I) to the total mass of fatty acid amides having a number of carbon atoms in the range from 16 to 24 (preferably octadecanamide) in the coating composition or the heat-sensitive recording layer is in the range from 1.2:1 to

13

4:1. In preferred embodiments, therefore, the mass of NKK used is at least slightly predominant (1.2:1) in comparison with the total mass of fatty acid amides used. Too great an excess of NKK (mass ratio greater than 4:1) is no longer advantageous, since in that case the positive properties and effects of the fatty acid amide (preferably octadecanamide) are no longer manifested in the desired way.

As already observed, a preferred coating composition or heat-sensitive recording layer of one aspect of the invention comprises octadecanamide (as the one or as one of plural fatty acid amides each having a number of carbon atoms in the range from 16 to 24). In preferred coating compositions or heat-sensitive recording layers of this kind, the ratio of the mass of the compound of formula (I) (NKK) to the mass of octadecanamide in the coating composition or the heat-sensitive recording layer is in the range from 1.2:1 to 4:1.

A preferred coating composition of one aspect of the invention or a heat-sensitive recording layer of one aspect of the invention, as defined above, preferably as defined above as being preferred, is characterized in that the ratio of the total mass of fatty acid amides having a number of 16 to 24 to the total mass of compounds selected from the group consisting of 1,2-diphenoxoethane (DPE) and ethylene glycol m-tolyl ether (EGTE) in the coating composition or the heat-sensitive recording layer is in the range from 4:1 to 1:2:1, preferably in the range from 1.5:1 to 1:2:1. Such ratios of the total amount of fatty acid amides having a number of carbon atoms in the range from 16 to 24 to the total mass of compounds selected from the group consisting of DPE and EGTE are particularly preferred since at the same time this achieves particularly high grease resistance and a low color development temperature. A low color development temperature is advantageous since no unduly large quantities of energy are needed in order to generate a color change. A high grease resistance increases the practical benefit and means that there are certain utilities for which such heat-sensitive recording materials become suitable at all. The fatty acid amides (preferably octadecanamide and/or N-(hydroxymethyl)octadecanamide) and DPE and/or EGTE interact synergistically, and so the required amount of fatty acid amides (preferably: octadecanamide) needed to achieve a stipulated grease resistance is comparatively low, in comparison with a situation where neither DPE nor EGTE is present. This dependency relationship between the parameters of grease resistance and color development temperature, which are critical for the practical benefit, and the mixing ratio of the fatty acid amide (preferably octadecanamide and/or N-(hydroxymethyl)octadecanamide) and also DPE and/or EGTE constituents is surprising in light of the prior art. If, in a coating composition of one aspect of the invention or a corresponding heat-sensitive recording layer, the total mass of fatty acid amides having a number of carbon atoms in the range from 16 to 24 to the total mass of DPE and/or EGTE that is chosen is too large, meaning a ratio of >4, for example, then it is no longer ensured in every case that the color development temperature is as low as desired. If, alternatively, too low a ratio is chosen, then it is no longer guaranteed in each individual case that the grease resistance will meet the requirements.

Particular preference is given to a coating composition of one aspect of the invention or a heat-sensitive recording layer of one aspect of the invention as defined above (preferably as identified above as being preferred), comprising

one or plural color developers, said one or at least one of the plural color developers being a compound of the formula (I)

14



one or plural dye precursors, octadecanamide and/or N-(hydroxymethyl)octadecanamide,

as sensitizer, 1,2-diphenoxoethane (DPE) and/or ethylene glycol m-tolyl ether (EGTE),

the ratio of the mass of the compound of the formula (I) to the mass of octadecanamide in the coating composition or the heat-sensitive recording layer being in the range from 1.2:1 to 4:1,

and the ratio of the total mass of octadecanamide and N-(hydroxymethyl)octadecanamide to the total mass of 1,2-diphenoxoethane (DPE) and ethylene glycol m-tolyl ether (EGTE)

in the coating composition or the heat-sensitive recording layer being in the range from 1.5:1 to 1:2:1.

A coating composition of one aspect of the invention of this kind or a heat-sensitive recording layer of one aspect of the invention of this kind unites advantages discussed above and is therefore, in particular, particularly grease resistant and has a comparatively low color development temperature, without any need for particularly high quantities of octadecanamide and/or N-(hydroxymethyl)octadecanamide in order to achieve the grease resistance.

A coating composition of one aspect of the invention or a heat-sensitive recording layer of one aspect of the invention (as defined above, preferably as identified above as being preferred) preferably comprises as sensitizer 1,2-diphenoxoethane (DPE) or a mixture of 1,2-diphenoxoethane (DPE) and ethylene glycol m-tolyl ether (EGTE). In such preferred coating compositions and heat-sensitive recording layers, therefore, DPE is present. With regard to preferred proportions, reference may be made to the observations above.

Preference is given to a coating composition of one aspect of the invention or a heat-sensitive recording layer of one aspect of the invention as defined above (preferably as identified above as being preferred), comprising, based on the oven-dry state,

8 to 30 percentage mass fractions (mass fractions expressed in %) of a total amount of one or plural color developers, said one or at least one of the plural color developers being a compound of the formula (I)



preferably 8 to 30 percentage mass fractions of the color developer of the formula (I), based in each case on the

## 15

total amount of the coating composition in the oven-dry state or of the heat-sensitive recording layer in the oven-dry state

and/or

4 to 16 percentage mass fractions of a total amount of one or plural dye precursors, based on the total amount of the coating composition in the oven-dry state or of the heat-sensitive recording layer in the oven-dry state

and/or

2.4 to 34 percentage mass fractions of a total amount of one or plural fatty acid amides each having a number of carbon atoms in the range from 16 to 24, preferably 2.4 to 34 percentage mass fractions of a total amount of one or more compounds selected from the group consisting of octadecanamide and N-(hydroxymethyl)octadecanamide, more preferably 2.4 to 34 percentage mass fractions of octadecanamide, based in each case on the total amount of the coating composition in the oven-dry state or of the heat-sensitive recording layer in the oven-dry state

and/or

2.4 to 34 percentage mass fractions of a total amount of one or plural fatty acid amides each having a number of carbon atoms in the range from 16 to 24, preferably 2.4 to 34 percentage mass fractions of a total amount of one or more compounds selected from the group consisting of octadecanamide and N-(hydroxymethyl)octadecanamide, more preferably 2.4 to 34 percentage mass fractions of octadecanamide, based in each case on the total amount of the coating composition in the oven-dry state or of the heat-sensitive recording layer in the oven-dry state

and/or

6 to 24 percentage mass fractions of a total amount of one or plural binders, preferably 6 to 24 percentage mass fractions of polyvinyl alcohol (PVA) (as particularly preferred binder), based in each case on the total amount of the coating composition in the oven-dry state or of the heat-sensitive recording layer in the oven-dry state

and/or

25 to 55 percentage mass fractions of a total amount of one or plural pigments, based on the total amount of the coating composition in the oven-dry state or of the heat-sensitive recording layer in the oven-dry state.

Particular preference is therefore given (in accordance with observations above) to a coating composition of the invention or a heat-sensitive recording layer of one aspect of the invention as defined above (preferably as identified above as being preferred), comprising, based on the oven-dry state,

8 to 30 percentage mass fractions of a total amount of one or plural color developers, said one or at least one of the plural color developers being a compound of the formula (I),

(I)



## 16

preferably 8 to 30 percentage mass fractions of the color developer of the formula (I), based in each case on the total amount of the coating composition in the oven-dry state or of the heat-sensitive recording layer in the oven-dry state,

4 to 16 percentage mass fractions of a total amount of one or plural dye precursors, based on the total amount of the coating composition in the oven-dry state or of the heat-sensitive recording layer in the oven-dry state,

2.4 to 34 percentage mass fractions of a total amount of one or plural fatty acid amides each having a number of carbon atoms in the range from 16 to 24, preferably 2.4 to 34 percentage mass fractions of a total amount of one or more compounds selected from the group consisting of octadecanamide and N-(hydroxymethyl)octadecanamide, more preferably 2.4 to 34 percentage mass fractions of octadecanamide, based in each case on the total amount of the coating composition in the oven-dry state or of the heat-sensitive recording layer in the oven-dry state,

as sensitizer, 2 to 8.5 percentage mass fractions of a total amount of one or more compounds selected from the group consisting of 1,2-diphenoxylethane and ethylene glycol m-tolyl ether, preferably 2 to 8.5 percentage mass fractions of 1,2-diphenoxylethane or 2 to 8.5 percentage mass fractions of a mixture of 1,2-diphenoxylethane and ethylene glycol m-tolyl ether, based in each case on the total amount of the coating composition in the oven-dry state or of the heat-sensitive recording layer in the oven-dry state,

6 to 24 percentage mass fractions of a total amount of one or plural binders, preferably 6 to 24 percentage mass fractions of polyvinyl alcohol (PVA), based in each case on the total amount of the coating composition in the oven-dry state or of the heat-sensitive recording layer in the oven-dry state, and

25 to 55 percentage mass fractions of a total amount of one or plural pigments, based on the total amount of the coating composition in the oven-dry state or of the heat-sensitive recording layer in the oven-dry state

with the proviso that for this particularly preferred coating composition or heat-sensitive recording layer, the ratio of the total mass of fatty acid amides having a number of carbon atoms in the range from 16 to 24 to the total mass of

compounds selected from the group consisting of 1,2-diphenoxylethane and ethylene glycol m-tolyl ether in the coating composition or the heat-sensitive recording layer is preferably in the range from 4:1 to 1.2:1. Analogous provisos apply preferably for embodiments of such a particularly preferred coating composition or heat-sensitive recording layer that result from combination with preferred embodiments and/or features as defined above or below in the appended claims.

It may be noted that the indications "based on the oven-dry state" and "in the oven-dry state" specify that the stated mass fractions of coating composition or heat-sensitive recording layer, respectively, relate to a measurement carried out on oven-dry material. The statements do not, however, mean that only oven-dry materials are defined; instead, a coating composition or a heat-sensitive recording layer also falls within the respective definition, for example, when it contains considerable amounts of liquid (e.g., water), provided that, after oven drying, a corresponding measurement results in total amounts of the relevant constituents that do fall within the respectively indicated ranges.

It is preferred in the invention if the heat-sensitive recording layer has a Bekk smoothness, determined according to

DIN 53107:2016-05 (title: Testing of paper and board—Determination of the smoothness by the Bekk method), of 100 to 1200 seconds, preferably of 150 to 1100 seconds.

As already observed above, one aspect of the invention also relates to a heat-sensitive recording material comprising a carrier substrate and a heat-sensitive recording layer of the invention. In a heat-sensitive recording material of the invention of this kind there are preferably one or plural interlayers disposed between carrier substrate and heat-sensitive recording layer. An interlayer of this kind preferably comprises pigments. The pigments may be organic pigments, inorganic pigments, or a mixture of organic pigments and inorganic pigments.

It is preferred in the invention if the surface mass of the interlayer is in the range from 5 to 20 g/m<sup>2</sup>, preferably in the range from 7 to 12 g/m<sup>2</sup>.

Where the interlayer comprises pigments, it is preferred in one aspect of the invention if the pigments are organic pigments, preferably organic hollow-body pigments.

In-house studies have shown the incorporation of organic pigments into the interlayer to be advantageous, because organic pigments exhibit high heat reflection capacity. Through increased heat reflection of the interlayer embodied with organic pigments, the response characteristics of the heat-sensitive recording layer with respect to heat are heightened, because the irradiated heat is reflected at least partly into the heat-sensitive recording layer, instead of being conducted to the carrier substrate. As a result, the sensitivity and the dissolution capacity of the heat-sensitive recording material are significantly increased and, furthermore, the printing speed in the thermal printer is boosted. Moreover, the energy consumption during the printing operation can be lowered, which is an advantage particularly in the case of mobile devices. Hollow-body pigments have air in their interior, and consequently they typically exhibit even greater heat reflection, and the sensitivity and the dissolution capacity of the heat-sensitive recording material can be increased further still.

Where the interlayer comprises pigments, it is preferred in an alternative embodiment of the invention if the pigments are inorganic pigments, preferably selected from the list consisting of calcined kaolin, silicon oxide, bentonite, calcium carbonate, aluminum oxide and boehmite.

Where inorganic pigments are incorporated into the interlayer situated between the recording layer and the substrate, these pigments are able, during formation of the written image, to accommodate the constituents of the heat-sensitive recording layer that have been liquefied by exposure to heat from the thermal head, and consequently they promote even more reliable and more rapid functioning of the heat-induced recording.

It is particularly advantageous if the inorganic pigments of the interlayer have an oil absorption value of at least 80 cm<sup>3</sup>/100 g and even better of 100 cm<sup>3</sup>/100 g, determined according to DIN EN ISO 787-5:1995-10 (title: General methods of test for pigments and extenders—Part 5: Determination of oil absorption value (ISO 787-5:1980); German version EN ISO 787-5:1995). On the basis of its high absorption reservoir in the hollow spaces, calcined kaolin has proven particularly suitable. Mixtures of plural inorganic pigments of different kinds may also be contemplated.

The choice of the proportion of organic to inorganic pigments produces a combination of the effects brought about by the two types of pigment. It is particularly advantageous if the pigment mixture consists of organic pigment with a mass fraction of 5 to 30% or, better still, at 8 to 20%, and of inorganic pigment at 95 to 70% or, better still, at 92

to 80%. Pigment mixtures of different organic pigments and/or inorganic pigments are advantageous in specific cases.

Preferred in one aspect of the invention is a heat-sensitive recording material, wherein the interlayer, optionally in addition to the inorganic and/or organic pigments, comprises at least one binder, preferably based on a synthetic polymer, with styrene-butadiene latex affording particularly good results. Polyvinyl alcohol (PVA) represents a further preferred binder. The use of a synthetic binder with admixture of at least one natural polymer, such as starch with particular preference, represents a particularly suitable embodiment of an interlayer. In the course of experiments with inorganic pigments it was also found that a binder-pigment ratio within the interlayer of between 3:7 and 1:9, based in each case on the percentage mass fraction in the interlayer, represents a particularly suitable embodiment.

Preference is given to a heat-sensitive recording material of one aspect of the invention, wherein no further layer is disposed on the side of the heat-sensitive recording layer that is facing away from the carrier substrate. In particular, therefore, the heat-sensitive recording layer of the heat-sensitive recording material of the invention does not carry a top coat. Such a top coat, though possible, is nevertheless not preferable, in particular because the heat-sensitive recording layer as set out above possesses particularly high grease resistance and consequently there is no longer any need for a top coat in order to bring about this quality.

Preference is given to a heat-sensitive recording material of one aspect of the invention, preferably a recording material of the invention as identified above as being preferred, wherein the carrier substrate consists of paper, synthetic paper, polymeric film, or an assembly of these materials. The technical effects associated with the present invention are largely independent of the carrier substrate, and so said substrate can be selected from a broad group of materials.

A particularly preferred carrier substrate, however, is a coating base paper which has not been surface-treated, since such a paper exhibits high recyclability and high environmental compatibility. A coating base paper which has not been surface-treated means a coating base paper which has not been treated in a sizing press or in a coating apparatus. Preferred polymeric films are films of polypropylene or other polyolefins. Also preferred in the invention are papers coated with one or more polyolefins (especially polypropylene).

In one especially preferred variant embodiment, the carrier substrate is a paper with a mass fraction of recycled fibers of at least 70%, based on the total pulp fraction in the paper.

A coating composition of one aspect of the invention and also a heat-sensitive recording layer of the invention each comprise one or more dye precursors (color formers). The use of color formers which are compounds of the fluoran type is preferred, preference being given to compounds selected from the group consisting of 3-diethylamino-6-methyl-7-anilinofluoran, 3-diethylamino-6-methyl-7-(3'-methylphenyl-amino)fluoran (6'-(diethylamino)-3'-methyl-2'-(m-tolylamino)-3H-spiro [isobenzofuran-1,9'-xanthen]-3-one; ODB-7), 3-di-n-pentylamino-6-methyl-7-anilinofluoran, 3-(diethylamino)-6-methyl-7-(3-methylphenylamino)fluoran, 3-di-n-butylamino-7-(2-chloroanilino)fluoran, 3-diethylamino-7-(2-chloroanilino)fluoran, 3-diethylamino-6-methyl-7-xylidinofluoran, 3-diethylamino-7-(2-carbomethoxyphenylamino)fluoran, 3-pyrrolidino-6-methyl-7-anilinofluoran, 3-pyrrolidino-6-

19

methyl-7-(4-n-butyl-phenylamino)fluoran, 3-piperidino-6-methyl-7-anilinofluoran, 3-N-n-dibutylamine-6-methyl-7-anilinofluoran (ODB-2), 3-(N-methyl-N-cyclohexyl)amino-6-methyl-7-anilinofluoran, 3-(N-methyl-N-propyl)amino-6-methyl-7-anilinofluoran, 3-(N-methyl-N-tetrahydrofurfuryl)amino-6-methyl-7-anilinofluoran, 3-(N-ethyl-N-isoamyl)amino-6-methyl-7-anilinofluoran, 3-(N-ethyl-N-tolyl)amino-6-methyl-7-anilinofluoran, 3-(N-ethyl-N-tetrahydrofuryl)amino-6-methyl-7-anilinofluoran, 3-(N-ethyl-N-isopentylamino)-6-methyl-7-anilinofluoran, 3-(N-ethyl-4-toluidino)-6-methyl-7-(4-toluidino)-fluoran, and 3-(N-cyclopentyl-N-ethyl)amino-6-methyl-7-anilinofluoran.

Likewise preferred are coating compositions or heat-sensitive recording layers of the invention which as dye precursors (color formers) comprise the compounds stated in paragraphs [0049] to [0052] of EP 2 923 851 A1.

Particularly preferred in one aspect of the invention is a coating composition of the invention, and a heat-sensitive recording layer of the invention, which use a dye precursor (color former) selected from the group consisting of 3-N-di-n-butylamine-6-methyl-7-anilinofluoran (ODB-2) and 3-(N-ethyl-N-isopentylamino)-6-methyl-7-anilinofluoran.

A coating composition of the invention and a heat-sensitive recording layer of the invention comprise one or plural color developers, said one or at least one of the plural color developers being NKK. Besides NKK there may be one or plural further color developers present, resulting overall in a color developer mixture. Preference is given to a coating composition of the invention and a heat-sensitive recording layer of the invention for which, in addition to a compound of the formula (I) (NKK) as first color developer, there is a further color developer which is a compound of the formula (II)



The compound of the formula (I) (NKK) is present preferably (but not necessarily) in a crystalline form, as already described above, which in the IR spectrum has an absorption band at  $3401 \pm 20 \text{ cm}^{-1}$ .

The compound of the formula (II) is the compound N-(4-methylphenylsulfonyl)-N'-(3-(4-methylphenylsulfonyloxy)phenyl)urea, which is already known, is sold under the name Pergafast® 201, and described for example in EP 1 140 515 B1. Pergafast® 201 is the most frequently used phenol-free color developer.

Surprisingly, the simultaneous presence of the compound of the formula (II) alongside the compound of the formula (I) (NKK) makes a further contribution to achieving a further increase in the grease resistance of a heat-sensitive recording layer of the invention and, respectively, of a corresponding heat-sensitive recording material of the invention. In relation to the resistance toward grease, a synergistic effect has been observed, which results when the compounds of the formula (I) and (II) are present simultaneously. Preferably, in coating compositions, heat-sensitive recording layers, and heat-sensitive recording materials of the invention, there is a mass ratio between the compound of the formula (I) and the compound of the formula (II) of

20

0.5:99.5 to 99.5:0.5. In-house studies have shown that for a mass fraction of less than 0.5% of the compound with the formula (I) or (II), based on the total mass of the compounds with the formula (I) and (II), the positive influence of the respective compound is not so greatly pronounced.

Particularly preferred in the invention are a coating composition of the invention, a heat-sensitive recording layer of the invention and also a heat-sensitive recording material of the invention, wherein the mass ratio between the compound of the formula (I) and the compound of the formula (II) is 10 35:65 to 65:35, preferably 40:60 to 60:40, more preferably 45:55 to 55:45.

Such mixtures produce a (further) synergistic effect in relation to improved resistance toward lanolin, and also, 15 moreover, an improved long-term stability.

As already observed above, certain objects forming a basis for one aspect of the present invention are achieved through the use of a fatty acid amide (as defined above and in the claims). For this use according to the invention, all of 20 the observations made above regarding (preferred) coating compositions, heat-sensitive recording layers, and heat-sensitive recording materials of the invention are valid correspondingly, mutatis mutandis.

It has already been observed earlier on above that the 25 invention achieves certain of the objects forming a basis for the present invention also through a method for producing a heat-sensitive recording material of the invention (as defined there and in the claims). In this respect as well, the observations above regarding (preferred) coating compositions, 30 heat-sensitive recording layers, and heat-sensitive recording materials of the invention are valid correspondingly, mutatis mutandis.

In a method of one aspect of the invention, the coating composition is preferably applied in an amount of 2.2 to 2.6 35 g/m<sup>2</sup> to the carrier substrate or to an interlayer disposed thereon. A coatweight of this kind is comparatively low by comparison with coating compositions from the prior art which are intended likewise to possess high grease resistance. In the context of the present invention it is possible to 40 achieve a high grease resistance with such a low coatweight for the reason that, owing to the synergistic interaction between the fatty acid amide having a number of carbon atoms in the range from 16 to 24 (preferably octadecanamide and/or N-(hydroxymethyl)octadecanamide) and the DPE and/or EGTE sensitizers, there is no need to use a large quantity of fatty acid amide which increases the grease resistance.

Preferred is a method of one aspect of the invention (as defined above and/or in the claims) for producing a heat-sensitive recording material (of one aspect of the invention), 50 having the following steps:

providing or producing

a carrier substrate with interlayer disposed thereon (in 55 each case preferably as described above as being preferred)

and also

a coating composition of the invention, applying the coating composition to the interlayer, 60 drying the applied coating composition, to give a heat-sensitive recording layer (of the invention) which is present together with the carrier substrate and the interlayer in the heat-sensitive recording material.

The heat-sensitive recording material produced with the method of the invention is a laminate which possesses at least one carrier substrate, an interlayer disposed thereon, and also a heat-sensitive recording layer disposed in turn on the interlayer. Regarding the advantages and the preferred

## 21

configurations of a heat-sensitive recording material with interlayer, see the observations earlier on above.

With regard to preferred configurations and combinations for a coating composition used in a method of the invention, the elucidations given above for the heat-sensitive recording materials of the invention are valid correspondingly (mutatis mutandis where appropriate), and vice versa.

The term "coating composition" in the context of the present invention and in agreement with the general understanding in the field of paper technology refers to coating materials comprising or consisting of pigments or matrix pigments, binders, and additives, said materials being applied to ("coated onto") the paper surface or to layers already applied to paper surfaces, using specific coating apparatus for surface finishing or surface modification of the paper. Papers produced in this way are referred to as "coated papers" and are notable, for example, for better tactile qualities. The term "coating composition" is therefore the generic term for all spreadable coating slips, preparations and/or solutions in the paper industry for the treatment, modification or finishing of a paper surface.

For the application of the coating composition to a carrier substrate or an interlayer, the skilled person knows of various coating technologies, examples including the following: blade coating, coating by film press, cast coating, curtain coating, knife coating, airbrush coating, or spray coating. All of these aforesaid known coating technologies are suitable for applying the coating compositions of the invention to a substrate, preferably a paper which comprises one or more preliminary coats or intermediate coats or else which comprises no preliminary coat or intermediate coat.

A further aspect of the present invention relates to products, preferably entry tickets, TITO tickets (ticket-in, ticket-out), flight, rail, ship or bus ticket, gaming ticket, car park ticket, label, till receipt, bank statements, self-adhesive label, medical and/or technical diagram paper, fax paper, security paper, or barcode labels, comprising a heat-sensitive recording material of the invention.

A further aspect of the present invention is the use of a heat-sensitive recording material of the invention as barcode label, self-adhesive lottery ticket, self-adhesive entry ticket, self-adhesive proof of purchase, self-adhesive label, self-adhesive entry ticket, entry ticket, TITO tickets (ticket-in, ticket-out), flight, rail, ship or bus ticket, gaming ticket, car park ticket, label, till receipt, bank statement, medical and/or technical diagram paper, fax paper, or security paper.

One aspect of the invention also relates to a method for producing a thermally printed, heat-sensitive recording material, having the following steps:

providing a heat-sensitive recording material of the invention (as defined above and in the claims, preferably as identified above as being preferred) or implementing the production method of the invention (as defined above and in the claims, preferably as identified above as being preferred), to give a heat-sensitive recording material,  
heat-treating the recording material, so that color developers and dye precursors react so as to develop a coloration.

In this case the fatty acid amide used having a number of carbon atoms in the range from 16 to 24 or the mixture of plural fatty acid amides used each having a number of carbon atoms in the range from 16 to 24, preferably octadecanamide and/or N-(hydroxymethyl)-octadecanamide, remains preferably in the solid state at the location of the heat treatment (the site at which in practice the thermal head acts).

## 22

The fatty acid amide used having a number of carbon atoms in the range from 16 to 24 or the mixture of plural fatty acid amides used each having a number of carbon atoms in the range from 16 to 24, preferably octadecanamide and/or N-(hydroxymethyl)-octadecanamide, therefore preferably does not melt and hence also does not act as a sensitizer.

The coloration formed is preferably part of a printed image, more particularly a printed graphic, an indicium, a pattern, or a recording.

## BRIEF DESCRIPTION OF THE DRAWINGS

The appended FIGS. 1, 2, 3, and 4 are graphic reproductions (fine drawings) of machine-generated original spectra and machine-generated original diffractograms, respectively.

FIG. 1 is a comparison of IR spectra in the wavenumber range from around 4000 to 2000  $\text{cm}^{-1}$  of the two crystalline forms of the compound of the formula (I);

FIG. 2 is a comparison of IR spectra in the wavenumber range from around 2400 to 400  $\text{cm}^{-1}$  of the two crystalline forms of the compound of the formula (I);

FIG. 3 is a comparison of IR spectra of the two crystalline forms of the compound of the formula (I); and

FIG. 4 is a comparison of X-ray powder diffractograms of the two crystalline forms of the compound of the formula (I).

## DETAILED DESCRIPTION OF THE PRESENTLY PREFERRED EMBODIMENTS

FIG. 1 shows a comparison of IR spectra in the wavenumber range from around 4000 to 2000  $\text{cm}^{-1}$  of the two crystalline forms of the compound of the formula (I). Depicted in the upper part and identified with a) is the IR spectrum of the crystalline form of the compound of the formula (I) used in the invention with a melting point of 175°C. Depicted in the lower part and identified with b) is the IR spectrum of the crystalline form of the compound of the formula (I) having a melting point of around 158°C.

FIG. 2 shows a comparison of IR spectra in the wavenumber range from around 2400 to 400  $\text{cm}^{-1}$  of the two crystalline forms of the compound of the formula (I). Depicted in the upper part and identified with a) is the IR spectrum of the crystalline form of the compound of the formula (I) used in the invention with a melting point of 175°C. Depicted in the lower part and identified with b) is the IR spectrum of the crystalline form of the compound of the formula (I) having a melting point of around 158°C.

FIG. 3 shows a comparison of IR spectra of the two crystalline forms of the compound of the formula (I). Depicted in the upper part and identified with a) is the IR spectrum of the crystalline form of the compound of the formula (I) used in the invention with a melting point of 175°C. Depicted in the lower part and identified with b) is the IR spectrum of the crystalline form of the compound of the formula (I) having a melting point of around 158°C.

FIG. 4 shows a comparison of X-ray powder diffractograms of the two crystalline forms of the compound of the formula (I). Depicted in the upper part and identified with a) is the X-ray powder diffractogram of the crystalline form of the compound of the formula (I) with a melting point of around 158°C. Depicted in the lower part and identified with b) is the X-ray powder diffractogram of the crystalline form of the compound of the formula (I) used in the invention having a melting point of 175°C.

23

Selected and preferred aspects of the invention are summarized below:

1. A coating composition for producing a heat-sensitive recording material or heat-sensitive recording layer, comprising

one or plural color developers, said one or at least one of the plural color developers being a compound of the formula (I)



(I)

one or plural dye precursors,  
one or plural fatty acid amides each having a number of carbon atoms in the range from 16 to 24,  
as sensitizer, one or more compounds selected from the group consisting of 1,2-diphenoxymethane and ethylene glycol m-tolyl ether.

2. The coating composition or heat-sensitive recording layer according to aspect 1, further comprising one or plural constituents from the group comprising

further sensitizers,  
pigments,  
dispersants,  
antioxidants,  
release agents,  
defoamers,  
light stabilizers,  
and  
brighteners.

3. The coating composition or heat-sensitive recording layer according to either of aspects 1 and 2, said one or one of the plural fatty acid amides having a number of carbon atoms in the range from 16 to 24

being octadecanamide and/or N-(hydroxymethyl)octadecanamide  
and/or

possessing a melting point which is greater than 103° C., preferably greater than 105° C.

4. The coating composition or heat-sensitive recording layer according to any of the preceding aspects,

the ratio of the total mass of the compound of the formula (I) to the total mass of fatty acid amides having a number of carbon atoms in the range from 16 to 24 in the coating composition or the heat-sensitive recording layer being in the range from 1.2:1 to 4:1

and/or

the ratio of the mass of the compound of the formula (I) to the mass of octadecanamide and/or N-(hydroxymethyl)octadecanamide in the coating composition or the heat-sensitive recording layer being in the range from 1.2:1 to 4:1.

5. The coating composition or heat-sensitive recording layer according to any of the preceding aspects, the ratio of the total mass of fatty acid amides having a number of carbon atoms in the range from 16 to 24 to the total mass of compounds selected from the group consisting of 1,2-diphenoxymethane and ethylene glycol m-tolyl ether in the coating composition or the heat-sensitive recording layer being in

24

the range from 4:1 to 0.8:1, preferably in the range from 2:1 to 1:1, more preferably in the range from 1.5:1 to 1:1, very preferably in the range from 1.5:1 to 1.2:1.

6. The coating composition or heat-sensitive recording layer according to any of the preceding aspects, comprising one or plural color developers, said one or at least one of the plural color developers being a compound of the formula (I)



(I)

one or plural dye precursors,  
octadecanamide and/or N-(hydroxymethyl)octadecanamide,  
as sensitizer, 1,2-diphenoxymethane and/or ethylene glycol m-tolyl ether,

the ratio of the mass of the compound of the formula (I) to the mass of octadecanamide and/or N-(hydroxymethyl)octadecanamide in the coating composition being in the range from 1.2:1 to 4:1,

and

the ratio of the total mass of octadecanamide and N-(hydroxymethyl)octadecanamide to the total mass of 1,2-diphenoxymethane and ethylene glycol m-tolyl ether

35 in the coating composition being in the range from 2:1 to 1:1, more preferably in the range from 1.5:1 to 1:1, very preferably in the range from 1.5:1 to 1.2:1.

7. The coating composition or heat-sensitive recording layer according to any of the preceding aspects, comprising  
40 as sensitizer 1,2-diphenoxymethane or a mixture of 1,2-diphenoxymethane and ethylene glycol m-tolyl ether.

8. A heat-sensitive recording material, comprising  
a carrier substrate  
and

a heat-sensitive recording layer according to any of aspects 1 to 7.

9. The heat-sensitive recording material, wherein  
one or plural interlayers are disposed between carrier  
substrate and heat-sensitive recording layer

and/or  
no further layer is disposed on the side of the heat-sensitive recording layer that faces away from the carrier substrate  
and/or

the carrier substrate consists of paper, synthetic paper,  
polymeric film, or an assembly of these materials.

10. The use of a fatty acid amide having a number of carbon atoms in the range from 16 to 24 or of a mixture of  
60 plural fatty acid amides each having a number of carbon atoms in the range of 16 to 24, preferably use of octadecanamide and/or N-(hydroxymethyl)octadecanamide, for increasing the grease resistance of a heat-sensitive recording material or a heat-sensitive recording layer, comprising

one or plural color developers, said one or at least one of the plural color developers being a compound of the formula (I)



one or plural dye precursors,  
and

as sensitizer, one or more compounds selected from the group consisting of 1,2-diphenoxymethane and ethylene glycol m-tolyl ether.

11. A method for producing a heat-sensitive recording material according to either of aspects 8 and 9 or a heat-sensitive recording layer, having the following steps:

providing or producing a carrier substrate and also a coating composition according to any of aspects 1 to 7, applying the coating composition to the carrier substrate or an interlayer disposed thereon, drying the applied coating composition, to give a heat-sensitive recording layer which is present together with the carrier substrate in a heat-sensitive recording material.

12. The method according to aspect 11, for producing a heat-sensitive recording material according to either of aspects 8 and 9, having the following steps:

providing or producing  
a carrier substrate with interlayer disposed thereon and also  
a coating composition according to any of aspects 1 to 7,  
applying the coating composition to the interlayer, drying the applied coating composition, to give a heat-sensitive recording layer which is present together with the carrier substrate and the interlayer in the heat-sensitive recording material.

13. A method for producing a thermally printed heat-sensitive recording material, having the following steps:

providing a heat-sensitive recording material according to either of aspects 8 and 9 or implementing the method according to either of aspects 11 and 12, to give a heat-sensitive recording material,  
heat-treating the recording material, so that color developers and dye precursors react so as to develop a coloration.

14. The method according to aspect 13, wherein the fatty acid amide used having a number of carbon atoms in the range from 16 to 24 or the mixture used of plural fatty acid amides each having a number of carbon atoms in the range from 16 to 24, preferably octadecanamide and/or N-(hydroxymethyl)octadecanamide, remains in the solid state at the location of the heat treatment.

## EXAMPLES

### Determining the Resistance of Heat-Sensitive Recording Materials to Lanolin:

For metrological capture of the resistance of a thermal printout on the heat-sensitive recording materials of the inventive examples and of the noninventive examples with respect to lanolin, test thermal printouts with a checkered black and white design were produced on each of the heat-sensitive recording materials under test, using an

Atlantek Model 400 "Thermal Response Test System" instrument from Global Media Instruments, LLC (USA), employing a thermal head having a resolution of 300 dpi and an energy per unit area of 16 mJ/mm<sup>2</sup>.

5 Following the production of the test thermal printouts with black and white checkering, and after a rest time of more than 5 minutes, a determination of the print density was carried out at three locations on the black-colored areas of the test thermal printouts, by a TECHKON® SpectroDens  
10 Advanced spectral densitometer. The mean was formed from the respective measurement values.

The test thermal printout produced on the heat-sensitive recording material under test was then coated with lanolin hand cream. After an exposure time of 5 and 10 minutes, 15 respectively, the lanolin was carefully dabbed off and then the treated thermal paper printout was stored at 23° C. and 50% humidity. After 4 hours and 24 hours, the thermal paper printout was removed, and again a determination of the print density was carried out at three locations on the black-colored areas of the test thermal printouts, by a TECHKON® SpectroDens Advanced spectral densitometer.

The mean was formed from the respective measurement values.

25 The resistance of the printed image in percent corresponds to the ratio of the mean of the print density of the black-colored areas before and after the treatment with lanolin and subsequent storage at 23° C. and 50% humidity, multiplied by 100.

### In-House Studies:

30 The results of measurement determined in in-house studies show that the print density of inventive examples decreases less than the print density of noninventive examples. The resistance of the printed image to lanolin, i.e., the grease resistance, is therefore higher for inventive examples than for noninventive examples, in which only a fatty acid amide or only 1,2-diphenoxymethane or ethylene glycol m-tolyl ether was used. The combination of stearamide (octadecanamide) or N-(hydroxymethyl)octadecanamide and 1,2-diphenoxymethane or ethylene glycol m-tolyl ether as sensitizer, used in accordance with the invention, 35 therefore has a synergistic effect.

In further in-house studies, preferred mixing ratios were determined for coating compositions comprising stearamide (octadecanamide) and 1,2-diphenoxymethane (DPE) as well. 45 In carrying out these experimental studies, a coating composition was produced which corresponds very largely to the aqueous application suspension of formulation 1 as per DE 10 2014 107 567 B3 (cf. paragraph [0060] therein). The total amount of octadecanamide (stearamide) and DPE in the in-house studies was 40 mass fractions (corresponding to the 40 mass fractions of sensitizer from formulation 1 from DE 10 2014 107 567 B3). Said 40 mass fractions were distributed in the in-house studies between the octadecanamide and DPE constituents, with the mixing ratios being varied. 50 Results of the studies are reported in table 1 below.

TABLE 1

|    | Mass fractions of<br>sensitizers Octadecanamide:<br>1,2-diphenoxymethane |       |       |       |      |
|----|--------------------------------------------------------------------------|-------|-------|-------|------|
|    | 20:20                                                                    | 23:17 | 25:15 | 27:13 |      |
|    | Experimental series I                                                    | I-1   | I-2   | I-3   |      |
| 65 | Print density before<br>lanolin exposure                                 | 1.16  | 1.23  | 1.21  | 1.13 |

TABLE 1-continued

|                                                                    | Mass fractions of sensitizers Octadecanamide: 1,2-diphenoxethane |       |       |       |
|--------------------------------------------------------------------|------------------------------------------------------------------|-------|-------|-------|
|                                                                    | 20:20                                                            | 23:17 | 25:15 | 27:13 |
| Print density after 5 min lanolin exposure and 4 h exposure time   | 0.70                                                             | 0.97  | 0.87  | 0.67  |
| Resistance/%                                                       | 60.3                                                             | 78.9  | 71.9  | 59.3  |
| Experimental series II                                             | II-1                                                             | II-2  | II-3  | II-4  |
| Print density before lanolin exposure                              | 1.15                                                             | 1.24  | 1.20  | 1.13  |
| Print density after 10 min lanolin exposure and 24 h exposure time | 0.18                                                             | 0.32  | 0.24  | 0.27  |
| Resistance/%                                                       | 15.7                                                             | 25.8  | 20.0  | 23.9  |

Outline composition for an inventive coating composition and for an inventive heat-sensitive recording layer:

Table 2 specifies a preferred outline composition for a coating composition of the invention and for a heat-sensitive recording layer of the invention. All of the data relate to measurement on oven-dry material; the actual coating composition or actual heat-sensitive recording layer may comprise liquid (especially water); it was therefore subjected to oven drying before determination of the mass fractions.

TABLE 2

|                                                                       | Mass fraction [%] |
|-----------------------------------------------------------------------|-------------------|
| N-[2-(3-Phenylureido)phenyl]benzenesulfonamide (NKK, color developer) | 8-30              |
| Dye precursor                                                         | 4-16              |
| Octadecanamide (fatty acid amide)                                     | 2.4-34            |
| 1,2-Diphenoxethane (sensitizer)                                       | 2-8.5             |
| Polyvinyl alcohol (PVA, binder)                                       | 6-24              |
| Pigments                                                              | 25-55             |
| Total                                                                 | 100               |

The percentage mass fractions reported in the right-hand column of table 2 add up to a total of 100%. Thus, while there have shown and described and pointed out fundamental novel features of the invention as applied to a preferred embodiment thereof, it will be understood that various omissions and substitutions and changes in the form and details of the devices illustrated, and in their operation, may be made by those skilled in the art without departing from the spirit of the invention. For example, it is expressly intended that all combinations of those elements and/or method steps which perform substantially the same function in substantially the same way to achieve the same results are within the scope of the invention. Moreover, it should be recognized that structures and/or elements and/or method steps shown and/or described in connection with any disclosed form or embodiment of the invention may be incorporated in any other disclosed or described or suggested form or embodiment as a general matter of design choice. It is the intention, therefore, to be limited only as indicated by the scope of the claims appended hereto.

The invention claimed is:

1. A coating composition for producing a heat-sensitive recording material, comprising:

at least one color developer, wherein at least one of the at least one color developer being a compound of formula (I)



wherein the compound of formula (I) is present in a crystalline form which in the IR spectrum has an absorption band at  $3401\pm20\text{ cm}^{-1}$ ,

at least one dye precursor;

20 at least one fatty acid amide each having a number of carbon atoms in a range from 16 to 24;

a sensitizer comprising at least one compound selected from the group consisting of 1,2-diphenoxethane and ethylene glycol m-tolyl ether; and

25 a ratio of a total mass of fatty acid amides having a number of carbon atoms in a range from 16 to 24 to a total mass of compounds selected from the group consisting of 1,2-diphenoxethane and ethylene glycol m-tolyl ether in the coating composition or the heat-sensitive recording layer being in a range from 4:1 to 1.2:1.

2. The coating composition as claimed in claim 1, further comprising at least one constituents from the group consisting of

30 a further sensitizer,  
a pigment,  
a dispersant,  
an antioxidant,  
a release agent,  
a defoamer,  
a light stabilizer, and  
a brightener.

3. The coating composition as claimed in claim 2,

35 wherein:  
the at least one fatty acid amide have a number of carbon atoms in a range from 16 to 24  
being octadecanamide and/or N-(hydroxymethyl)octadecanamide and/or

40 possessing a melting point which is greater than  $103^\circ\text{ C}$ .

4. The coating composition as claimed in claim 3, wherein a ratio of the mass of the compound of the formula (I) to a total mass of fatty acid amides having the number of carbon atoms in a range from 16 to 24 in the coating composition or the heat-sensitive recording layer being in a range from 1.2:1 to 4:1  
55 and/or

5. The coating composition as claimed in claim 1, to the mass of octadecanamide and/or N-(hydroxymethyl) octadecanamide in the coating composition being in a range from 1.2:1 to 4:1.

60 5. The coating composition as claimed in claim 1, wherein a ratio of a total mass of fatty acid amides having a number of carbon atoms in the range from 16 to 24 to a total mass of compounds selected from the group consisting of 1,2-diphenoxethane and ethylene glycol m-tolyl ether in the coating composition being in a range from 1.5:1 to 1.2:1.

29

6. The coating composition as claimed in claim 1, comprising as sensitizer 1,2-diphenoxoethane or a mixture of 1,2-diphenoxoethane and ethylene glycol m-tolyl ether.

7. The coating composition as claimed in claim 1, the at least one fatty acid amides having a number of carbon atoms in a range from 16 to 24 being octadecanamide and/or N-(hydroxymethyl)octadecanamide and/or possessing a melting point which is greater than 103° C. 5

8. A coating composition for producing a heat-sensitive recording material or heat-sensitive recording layer, comprising 10

at least one color developer, wherein at least one of the at least one color developers being a compound of a formula (I) 15



wherein the compound of formula (I) is present in a crystalline form which in the IR spectrum has an absorption band at  $3401\pm20\text{ cm}^{-1}$ , 30

at least one dye precursor; octadecanamide and/or N-(hydroxymethyl)octadecanamide;

a sensitizer comprising, 1,2-diphenoxoethane and/or ethylene glycol m-tolyl ether, 35

wherein a ratio of a mass of the compound of the formula (I) to a mass of octadecanamide and/or N-(hydroxymethyl)octadecanamide in the coating composition being in a range from 1.2:1 to 4:1,

and 40 a ratio of a total mass of octadecanamide and N-(hydroxymethyl)octadecanamide to the total mass of 1,2-diphenoxoethane and ethylene glycol m-tolyl ether in the coating composition being in a range from 1.5:1 to 1.2:1.

9. A heat-sensitive recording material, comprising:

a carrier substrate; and

a heat-sensitive recording layer comprising:

at least one color developer, wherein at least one of the at least one color developer being a compound of formula (I) 50



wherein the compound of formula (I) is present in a crystalline form which in the IR spectrum has an absorption band at  $3401\pm20\text{ cm}^{-1}$ , 65

at least one dye precursor;

30

at least one fatty acid a amide each having a number of carbon atoms in a range from 16 to 24;

a sensitizer comprising at least one compound selected from the group consisting of 1,2-diphenoxoethane and ethylene glycol m-tolyl ether; and

a ratio of a total mass of fatty acid amides having a number of carbon atoms in a range from 16 to 24 to a total mass of compounds selected from the group consisting of 1,2-diphenoxoethane and ethylene glycol m-tolyl ether in the coating composition or the heat-sensitive recording layer being in a range from 4:1 to 1.2:1.

10. The heat-sensitive recording material as claimed in claim 9, further comprising

at least one interlayer disposed between the carrier substrate and the heat-sensitive recording layer

and/or wherein no further layer is disposed on a side of the heat-sensitive recording layer that faces away from the carrier substrate

and/or wherein the carrier substrate consists of paper, synthetic paper, polymeric film, or an assembly of these materials.

11. A heat sensitive recording material comprising: a carrier substrate; and a heat-sensitive recording layer, comprising: at least one color developer, wherein at least one of the at least one color developer being a compound of formula (I) 30



wherein the compound of formula (I) is present in a crystalline form which in the IR spectrum has an absorption band at  $3401\pm20\text{ cm}^{-1}$ ,

at least one dye precursor; at least one fatty acid amide each having a number of carbon atoms in a range from 16 to 24 and comprising octadecanamide and/or (N-hydroxymethyl)octadecanamide;

as a sensitizer, comprising at least one compound selected from the group consisting of 1,2-diphenoxoethane and ethylene glycol m-tolyl ether; and

a ratio of a total mass of fatty acid amides having a number of carbon atoms in a range from 16 to 24 to a total mass of compounds selected from the group consisting of 1,2-diphenoxoethane and ethylene glycol m-tolyl ether in the coating composition or the heat-sensitive recording layer being in a range from 4:1 to 1.2:1.

12. A method for producing a heat-sensitive recording material, comprising

providing or producing a carrier substrate and also a coating composition comprising:

at least one color developer, wherein at least one of the at least one color developers being a compound of formula (I)

31



(I)

5  
10  
15  
20  
25  
30  
35

wherein the compound of formula (I) is present in a crystalline form which in the IR spectrum has an absorption band at  $3401\pm20\text{ cm}^{-1}$ ,  
 at least one dye precursor;  
 at least one fatty acid amide each having a number of carbon atoms in a range from 16 to 24;  
 a sensitizer comprising at least one compound selected from the group consisting of 1,2-diphenoxymethane and ethylene glycol m-tolyl ether; and  
 a ratio of a total mass of fatty acid amides having a number of carbon atoms in a range from 16 to 24 to a total mass of compounds selected from the group consisting of 1,2-diphenoxymethane and ethylene glycol m-tolyl ether in the coating composition being in a range from 4:1 to 1.2:1;  
 applying the coating composition to the carrier substrate or an interlayer disposed thereon;  
 drying the applied coating composition, to give a heat-sensitive recording layer on the carrier substrate as the heat-sensitive recording material.

13. The method as claimed in claim 12, comprising:  
 providing or producing the carrier substrate with the interlayer disposed thereon applying the coating composition to the interlayer; and  
 drying the applied coating composition, to give a heat-sensitive recording layer on the interlayer which is on the carrier substrate as the heat-sensitive recording material.

14. A method for producing a thermally printed heat-sensitive recording material, comprising:  
 providing a heat-sensitive recording material comprising:  
 a carrier substrate; and

32

a heat-sensitive recording layer comprising:  
 at least one color developer, wherein at least one of the at least one color developer being a compound of formula (I)

(I)  
15  
20  
25  
30  
35

wherein the compound of formula (I) is present in a crystalline form which in the IR spectrum has an absorption band at  $3401\pm20\text{ cm}^{-1}$ ,  
 at least one dye precursor;  
 at least one fatty acid amide each having a number of carbon atoms in a range from 16 to 24;  
 a sensitizer comprising at least one compound selected from the group consisting of 1,2-diphenoxymethane and ethylene glycol m-tolyl ether; and  
 a ratio of a total mass of fatty acid amides having a number of carbon atoms in a range from 16 to 24 to a total mass of compounds selected from the group consisting of 1,2-diphenoxymethane and ethylene glycol m-tolyl ether in the heat-sensitive recording layer being in a range from 4:1 to 1.2:1; and  
 heat-treating the heat-sensitive recording material, so that the at least one color developer and the at least one dye precursor reacts so as to develop a coloration.

15. The method as claimed in claim 14, wherein the at least one fatty acid amide remains in the solid state at the location of the heat treating.

16. A heat-sensitive recording material, comprising a carrier substrate and a heat sensitive recording later formed from the coating composition in claim 1.

\* \* \* \* \*